

Oct. 1, 1935.

N. H. MAGEE ET AL

2,015,903

PROCESS FOR COLORING ETCHINGS ON GLASSWARE

Filed Dec. 22, 1931



Fig. 1.



Fig. 2.



Fig. 3.



Fig. 4.



Fig. 5.



Fig. 6.

INVENTORS,

Norman H. Magee and  
John A. Patterson Jr.  
by their attorney,  
J. Edward Shabaud.

## UNITED STATES PATENT OFFICE

2,015,903

PROCESS FOR COLORING ETCHINGS ON  
GLASSWARE

Norman H. Magee and John A. Patterson, Jr.,  
Philadelphia, Pa., assignors to John M. Maris  
Company, Inc., a corporation of Pennsylvania

Application December 22, 1931, Serial No. 582,647

4 Claims. (Cl. 41—41)

Our invention relates to new and useful improvements in the art of producing colored etchings on glassware.

Ordinarily, when it is desired to color etchings upon glassware, which etchings have been produced either by grinding or by the use of hydrofluoric acid, some colored opaque material, such as enamel is used to fill in the ground-in or chemically etched markings on the glass surface, to make the same visible. Such coloring materials, used to fill in the said markings, lack permanency, and are worn off in ordinary use, during washing or handling or in the event of contact with some corrosive chemicals.

It is our object to provide a chemical process for coloring etchings upon glassware, which will eliminate much labor in coloring of the markings, and at the same time, produce a form of coloring in the markings which becomes a permanent part of the glassware.

Generally speaking, after first grinding or chemically etching the desired markings in design, lettering, etc., on the glassware, through some wax or other protective coating, we immerse the glassware in a bath containing some metallic salts followed by a bath containing one or more appropriate precipitating agents, which leaves the precipitate lodged within the etched markings as an insoluble metallic inorganic compound or compounds, or mixtures. This is followed by rinsing in water and removing the protective coating, then by dehydrating the lodged precipitates, to cause a greater adherence of the same to the glass. We select such metallic salt or salts and appropriate precipitating agent or agents as will give us the desired color or shade of color.

The inorganic metallic compounds adapted for the purposes of our process, may be listed as oxides or hydroxides, silicates, chromates, sulphates, carbonates, including also barium sulfate, ferrous ferricyanide, ferric ferrocyanide, silver arsenate, silver arsenite, silver chloride, silver bromide, silver iodide, lead basic carbonate.

Below we have listed the various inorganic metallic compounds, suitable for use in our process. Opposite each compound, we have given the corresponding color of the resulting precipitate formed, as follows:

50 *The oxides or hydroxides*

|                                  |               |
|----------------------------------|---------------|
| Chromic                          | Green         |
| Lead (litharge, PbO)             | Yellow or red |
| Magnesium                        | White         |
| Tin (stannic, SnO <sub>2</sub> ) | White         |
| Iron                             | Red or black  |

55 *The carbonates*

|          |       |
|----------|-------|
| Cobaltus | Red   |
| Barium   | White |

*The sulfides*

|                                            |                |
|--------------------------------------------|----------------|
| Copper                                     | Black          |
| Iron                                       | Black          |
| Mercury                                    | Black or red   |
| Antimony (Sb <sub>2</sub> S <sub>3</sub> ) | Black or brown |
| Antimony (Sb <sub>2</sub> S <sub>5</sub> ) | Orange         |
| Arsenic (As <sub>2</sub> S <sub>2</sub> )  | Red            |
| Arsenic (As <sub>2</sub> S <sub>3</sub> )  | Yellow         |
| Arsenic (As <sub>2</sub> S <sub>5</sub> )  | Yellow         |
| Cadmium                                    | Yellow         |
| Nickel                                     | Black          |
| Lead                                       | Black or brown |

*The chromates*

|         |        |
|---------|--------|
| Lead    | Yellow |
| Silver  | Red    |
| Mercury | Red    |

And in addition,

|                      |            |
|----------------------|------------|
| Barium sulfate       | White      |
| Ferrous ferricyanide | Light blue |
| Ferric ferrocyanide  | Dark blue  |
| Silver arsenate      | Red        |
| Silver arsenite      | Yellow     |
| Silver chloride      | White      |
| Silver bromide       | Yellow     |
| Silver iodide        | Yellow     |
| Lead basic carbonate | White      |

Also the silicates of: Aluminum, bismuth, boron, 30  
cadmium, calcium, chromium, cobalt, copper,  
iron, lead, magnesium, manganese, mercury,  
nickel, silver, tin, titanium, and zinc, may be  
used.

More specifically, let us assume it is desired to 35  
produce yellow markings on glassware, then our  
process for producing a yellow coloring of hydro-  
fluoric acid etched markings may be stated as  
follows:

The glassware is first coated all over with some 40  
protective coating, as wax, to protect the parts  
of the glass surface which are not exposed for  
the etched markings, when the glass piece is im-  
mersed in any of the various chemical baths used  
in our process. After the design or lettering to 45  
be marked upon the glass, is either ground there-  
on, through the protective coating or the lines of  
the design or lettering cut through the said coat-  
ing, merely to expose the glass surface in lines  
corresponding to the design or lettering, for sub- 50  
sequent etching by the usual bath of hydrofluoric  
acid, solution, then the glass article, so marked  
through its solution coating, is given a bath of  
hydrofluoric acid solution and is left long enough  
immersed to lodge certain fluorides along the 55  
lines of the markings, which have been either  
ground in through the coating, or where the glass  
has been merely exposed through the use of a  
needle or stylus in making the markings through  
the coating. In the latter case, which is the 60

usual way of forming the markings for subsequent etchings by the use of a hydrofluoric acid solution, the glassware is immersed in a hydrofluoric acid solution to form the etchings in the lines of the markings and is next rinsed in cold water, so as not to disturb the protective coating, yet leave some fluorides lodged in the etchings, and after so rinsing the glass article, it is given a second treatment by immersing again in a hydrofluoric acid frosting solution containing ammonium salts to form an etched frosting along the markings. In the case where the markings are ground into the glass through the protective coating this first bath of hydrofluoric acid solution is omitted, but the subsequent treatment is the same, whether the markings were formed by grinding in, or were formed by the use of a stylus and etched in by hydrofluoric acid. Before proceeding further, the glassware is rinsed. Then follows, in either case, the next step which consists in immersing the glassware in a solution of lead acetate, containing a slight excess of acetic acid. The glassware is held long enough in this last mentioned solution to dissolve the fluorides remaining upon the etched lines of the glass and to wet these lines in the glass with the lead salts formed. The glassware is next rinsed in cold water and subsequently immersed in a solution of ammonium bichromate, forming insoluble lead chromate, as a precipitate, lodged within the said etched markings. After being in this last bath long enough to attain the desired results, ascertained by practice, the glassware is allowed to dry off in the air long enough to dehydrate the precipitate causing it to adhere more firmly to the glass, after which the glassware is washed off in boiling hot water or other suitable liquid to remove the protective coating, and then the glassware is in a finished condition to be wiped dry, leaving yellow markings practically, permanently fixed upon the glassware.

In a similar way, the chemist who is familiar with this art will readily understand how to get any other desired color by using the suggestions above tabulated in selecting the proper metallic salt and its corresponding precipitant for the color desired, as he carries out a like sequence of steps, as above described for producing the yellow markings on the glassware.

In order to graphically portray the various steps taken, as well as to indicate the nature of the chemical baths, through which the glass article is passed, to produce the anchored colored precipitates, at the etchings, we have shown in Figure 1, a perspective view of a glass plate 10, covering with a protective coating 11, through which a broad marking 12 has been scratched, to expose the glass surface at 13. In Figure 2, the dish 14 is shown in section, to hold the glass plate 10, in a bath 15 of solution containing hydrofluoric acid as the usual etching bath, to form the initial etching, where 16 represents the layer of fluorides, constituting this etching.

In Figure 3 the dish 14 is shown in section, to hold the glass plate 10, in a different bath 17, or one of solution of hydrofluoric acid mixed with ammonium salts, thereby producing the microscopic pits indicated at 18, in this Figure 3, the modified etching layer being indicated at 19. In Figure 4, the dish 14 is shown in section to hold the glass plate 10 in a bath 20, containing a metallic salt, which chemically combines with the fluorides formed in the previous baths, the changed etching being here marked 21.

Figure 5 shows the dish 14 in section holding

the plate 10, in a bath 22, of solution containing an appropriate reagent to the metallic salt used in bath 20, the further changed and colored etching being marked 23. Figure 6 is a perspective view of the finished plate 10, with a colored and anchored etching 23, having the protective coating 11 removed.

Inasmuch as modifications of our process of forming colored etchings on glassware can be used without departing from the spirit and scope of our invention, we wish to include all which come within the purview of the following claims.

We claim:

1. The process of chemically treating a glass surface to produce anchored colored etchings thereon, which includes the following steps; first, covering the surface of the glass with some protective coating, as a suitable wax, then making markings of the desired design or lettering thru the said coating to expose the surface of the glass to be etched, then immersing the glass in a bath of solution containing hydrofluoric acid, as the usual etching bath, to form the initial etching at the said markings, next following this initial etching with the production of a chemical and physical anchorage for the subsequently produced colored precipitates by means of giving the glass a bath of solution of hydrofluoric acid mixed with ammonium salts, whereby producing a pitted surface at the said markings, together with added fluorides, following this pitting of the glass surface with a bath containing metallic salt, and subsequently immersing the said glass in a bath containing an appropriate reagent to the metallic salt used, whereby the colored precipitate so produced, reaches down into the said pitted surface to be more firmly secured against wear.

2. The process of chemically treating a glass surface to produce anchored colored etchings thereon, which includes the following steps: first, covering the surface of the glass with some protective coating, as a suitable wax, then making markings of the desired design or lettering through the said coating to expose the surface of the glass to be etched, then immersing the glass in a bath of solution containing hydrofluoric acid, as the usual etching bath, to form the initial etching at the said markings, next following this initial etching with the production of a chemical and physical anchorage for the subsequently produced colored precipitates by means of giving the glass a bath of solution of hydrofluoric acid mixed with ammonium salts, whereby producing a pitted surface at the said markings together with added fluorides, following this pitting of the glass surface with a bath containing metallic oxide, and subsequently immersing the said glass in a bath containing an appropriate reagent to the metallic oxide used, whereby the colored precipitate so produced, reaches down into the said pitted surface to be more firmly secured against wear.

3. The process of chemically treating a glass surface to produce anchored colored etchings thereon, which includes the following steps: First, covering the surface of the glass with some protective coating, as a suitable wax, then making markings of the desired design or lettering through the said coating to expose the surface of the glass to be etched, then immersing the glass in a bath of solution containing hydrofluoric acid, as the usual etching bath, to form the initial etching at the said markings, next following this initial etching with the production of a chemical

and physical anchorage for the subsequently produced colored precipitates by means of giving the glass a bath of solution of hydrofluoric acid mixed with ammonium salts, whereby producing 5 a pitted surface at the said markings, together with added fluorides, following this pitting of the glass surface with a bath containing metallic carbonate, and subsequently immersing the said glass in a bath containing an appropriate reagent 10 to the metallic carbonate used, whereby the colored precipitate so produced, reaches down into the said pitted surface to be more firmly secured against wear.

4. The process of chemically treating a glass 15 surface to produce anchored colored etchings thereon, which includes the following steps: first, covering the surface of the glass with some protective coating, as a suitable wax, then making markings of the desired design or lettering 20 through the said coating to expose the surface of

the glass to be etched, then immersing the glass in a bath of solution containing hydrofluoric acid, as the usual etching bath, to form the initial etching at the said markings, next following this initial etching with the production of a chemical and physical anchorage for the subsequently produced colored precipitates by means of giving the glass a bath of solution of hydrofluoric acid mixed with ammonium salts, whereby producing a 5 pitted surface at the said markings, together with added fluorides, following this pitting of the glass surface with a bath containing metallic silicate, and subsequently immersing the said glass in a bath containing an appropriate reagent to the metallic silicate used, whereby the colored precipitate so produced, reaches down into the said 10 pitted surface to be more firmly secured against wear. 15

NORMAN H. MAGEE.  
JOHN A. PATTERSON, JR. 20